

## 1

3,460,953

PROCESS FOR DEPOSITING BRASSLIKE COATINGS  
AND COMPOSITION THEREFOR

Norbert C. Schwartz, Homer, N.Y., assignor to Pennsalt Chemical Corporation, Philadelphia, Pa., a corporation of Pennsylvania

No Drawing. Filed May 27, 1966, Ser. No. 553,286

Int. Cl. C23b 5/36; C09d 5/00

U.S. Cl. 106—1

10 Claims

## ABSTRACT OF THE DISCLOSURE

An immersion process and a composition for applying a brasslike finish to steel by immersing steel in a bath comprising copper, nickel, and tin, together with a complexing agent of the group of boric acid and citric acid, and an enhancing agent of the group of glutaric acid, succinic acid, glycolic acid, their anhydrides, and their water soluble salts.

This invention relates to immersion electrolytic plating, and more particularly to electrolytes therefor.

An important object of the invention is to provide plating electrolytes for use in plating brasslike coatings on objects, which coatings are substantially similar in appearance to those generally known as "liquor finish," and employing a tertiary system of cupric, nickelous and stannous salts.

Another important object of the invention is to provide new and useful immersion electrolytic plating electrolytes containing new additions, functioning as complexing and chelating agents for the plating of a metal or metals.

Still another important object of the invention is to provide a new and useful immersion electroplating electrolyte, containing enhancing and modifying agents for the complexing and chelating agents.

The added agents improve the thickness, density, adhesion, appearance and anti-tarnishing characteristics of the plated objects.

In addition, an important object of the invention is to provide immersion electrolytic plating electrolytes which tend to slow the build-up of iron salts in the electrolytes, whereby the useful lives of the electrolytes are lengthened.

Another important object of the invention is to provide new and useful immersion electrolytic plating electrolytes which contain low to moderate cost compounds which are readily obtainable and which may be incorporated in a sulfuric acid-containing electrolyte by conventional steps, whereby the electrolytes may be produced and marketed at moderate prices.

An additional object of the invention is to provide several chemical classes of brightening agents which function in these electrolytes to enhance, improve, and brighten the coating obtained.

Other objects and advantages of the invention will be apparent during the course of the following detailed description of the invention.

A preferred example of my complexing and chelating agents is boric acid, and preferred examples of my enhancing and modifying agents are glutaric anhydride, sodium glycolate and succinic anhydride. Examples of brightening agents include 3-amino-1H-1, 2,4-triazole and 2-butyne-1, 4-diol. Examples of the plating salts are

## 2

those of copper, nickel and tin, either employed together, any two, or separately. An example of the objects to be placed are iron or steel wires or rods.

Numerous classes of chemical compounds have been found to enhance, improve, and brighten the deposited coating. Among these are: magnesium salts, for example magnesium chloride; short chain monobasic carboxylic acids, for example formic acid, or the corresponding sodium or potassium salts, for example sodium acetate and sodium formate; fluoroboric acid and its salts, for example sodium fluoroborate; benzimidazoles, for example 2-methylbenzimidazoles; aldehydes, for example paraformaldehyde; triazoles, for example 3-amino-1H-1,2,4-triazole; piperazines, for example 2-methylpiperazine; and acetylenic diols, for example 2-butyne-1,4-diol. It is, of course, obvious that these are specific examples that the general classes of compounds including carboxylic acids, fluoroboric acids, aldehydes, acetylenic diols, triazoles, benzimidazoles, piperazines, and related classes of compounds would tend to function to enhance, improve, and brighten coating to some extent.

Although I consider glutaric anhydride, sodium glycolate and succinic anhydride as my preferred enhancing and modifying agents, I have experimented with other agents including citric acid, gluconic acid, succinic acid, ethylenediamine tetracetic acid. These are only specific examples, the series of related acids including tartaric, fumaric, maleic, propionic, butyric, valeric, and other similar acids are adaptable. I have discovered that, especially, glutaric anhydride, sodium glycolate and succinic anhydride, in combination with for example, boric acid, citric acid or hydroxy acetic acid, impart synergistic effects to the complexing and chelating agents employed, since the qualities of the plating are enhanced over those where any one member of one group or one member of the other group are employed.

In the following examples of formulae, the preferred grade of boric acid is U.S.P.; of glutaric anhydride, the technical grade and sodium glycolate, the purified grade. The sulfuric acid of the electrolyte is preferably conventional 66° Baumé in tap water, with the grades of the salts of the plating metals those commonly used in immersion electrolytic plating electrolytes.

Since very superior platings result from the use of boric acid associated with glutaric anhydride in my formulations, the following Example 1 is given.

## EXAMPLE 1

50 Consisting of a dry admixture of the following composition to be used in aqueous solution of suitable concentration to produce an immersion coating on steel objects, the percentages of specific ingredients in this and the other examples are by weight, except as noted herein-  
55 after.

|                                 | Specific Example, percent | Specific Dry Admixture, percent |
|---------------------------------|---------------------------|---------------------------------|
| 60 Boric acid.....              | 5.03                      | 50.3                            |
| Glutaric anhydride.....         | 1.05                      | 10.5                            |
| Copper sulfate.....             | 0.55                      | 5.5                             |
| Nickel sulfate.....             | 3.00                      | 30.0                            |
| Stannous chloride (anhyd.)..... | 0.37                      | 3.7                             |
| 66° Bé sulfuric acid.....       | 90.00                     |                                 |
| Water.....                      | 100.00                    | 100.0                           |

In place of glutaric anhydride, I may substitute sodium glycolate as follows:

## EXAMPLE 2

|                            | Specific Example, percent | Specific Dry Admixture, percent |
|----------------------------|---------------------------|---------------------------------|
| Boric acid                 | 4.0                       | 38.1                            |
| Sodium glycolate           | 2.0                       | 19.0                            |
| Copper sulfate             | 1.0                       | 9.5                             |
| Nickel sulfate             | 3.0                       | 28.6                            |
| Stannous chloride (anhyd.) | 0.5                       | 4.8                             |
| Sulfuric acid              | 0.5                       |                                 |
| Water                      | 89.0                      |                                 |
|                            | 100.0                     | 100.0                           |

Instead of the glycolate or anhydride, I may substitute citric acid, as follows:

## EXAMPLE 3

|                            | Specific Example, percent | Specific Dry Admixture, percent |
|----------------------------|---------------------------|---------------------------------|
| Boric acid                 | 3.0                       | 28.6                            |
| Citric acid                | 3.0                       | 28.6                            |
| Copper sulfate             | 1.0                       | 9.5                             |
| Nickel sulfate             | 3.0                       | 28.6                            |
| Stannous chloride (anhyd.) | 0.5                       | 4.8                             |
| Sulfuric acid              | 0.5                       |                                 |
| Water                      | 89.0                      |                                 |
|                            | 100.0                     | 100.0                           |

Or, in place of the above, I may substitute succinic acid, as follows:

## EXAMPLE 4

|                            | Specific Example, Percent | Specific Dry Admixture, Percent |
|----------------------------|---------------------------|---------------------------------|
| Boric acid                 | 4.0                       | 38.1                            |
| Succinic acid              | 2.0                       | 19.0                            |
| Copper sulfate             | 1.0                       | 9.5                             |
| Nickel sulfate             | 3.0                       | 28.6                            |
| Stannous chloride (anhyd.) | 0.5                       | 4.8                             |
| Sulfuric acid              | 0.5                       |                                 |
| Water                      | 89.0                      |                                 |
|                            | 100.0                     | 100.0                           |

Alternatively, in place of succinic acid, I may substitute diglycolic acid, Rochelle salt, gluconic acid, salicylic acid, ethylenediamine tetraacetate, or sodium chloride.

As a reduction to practice of the process and practice exemplified by the formulation containing boric acid and glutaric anhydride, 100 milliliters of an eight-percent by weight solution of the electrolyte of Example 1 was prepared. Mild steel panels 20 gauge, cold rolled, 1½ by 2 inches were coated by immersion in this solution for three minutes, after about 65 panels had been coated, 4 percent by weight of Example 1 was added to replenish the bath. The color and brightness of the coating was found to be excellent after 728 panels had been coated in 100 milliliters of this solution in this manner. The solution was analyzed before use and after 728 panels for boric acid by manitol titration, nickel by dimethyl glyoxime, copper by thiosulfate titration after separation on aluminum foil, tin by precipitation from nitric acid solution and iron by cupferron precipitation, the steps resulting in the following:

|            | Before Use, Percent          | After 728 Panels, Percent |
|------------|------------------------------|---------------------------|
| Boric acid | 4.57                         | 4.48                      |
| Copper     | 0.0038 as $Cu^{2+}$          | (1)                       |
| Nickel     | 4.34 as $NiSO_4 \cdot 6H_2O$ | 3.48                      |
| Tin        | 0.062 as $Ti^{2+}$           | .961                      |
| Iron       | None                         | .193                      |

<sup>1</sup> Negligible.

After 200 panels, the copper indicated by titration was 0.0095%, and after 300 panels, 0.025% expressed as metallic copper. Variations observed may be partly due to the complexity of the analytical procedure.

It was observed that the incorporation of sodium chlo-

ride in an immersion plating bath consisting of boric acid, nickel sulfate, copper sulfate, and stannous chloride modifies, enhances, and brightens the deposited coating. This concept is illustrated in Example 5 in which the ratios are merely specific examples of the general principle.

## EXAMPLE 5

|                            | Specific Example, Percent | Specific Dry Admixture, Percent |
|----------------------------|---------------------------|---------------------------------|
| Boric acid                 | 5.0                       | 47.6                            |
| Sodium chloride            | 1.0                       | 9.5                             |
| Copper sulfate             | 1.0                       | 9.5                             |
| Nickel sulfate             | 3.0                       | 28.6                            |
| Stannous chloride (anhyd.) | 0.5                       | 4.8                             |
| Water                      | 89.5                      |                                 |
|                            | 100.0                     | 100.0                           |

The sodium chloride may be of any grade from U.S.P. XV to table salt.

Three modifications of the foregoing formulae are contained in Examples 6 to 8. One illustrates the modification, improvement, enhancement, and brightening produced by the incorporation of succinic anhydride in an immersion plating bath consisting of citric acid, copper, nickel and stannous salts. The second and third are examples of the modification, improvement and enhancement resulting from the incorporation of either hydroxy acetic acid, or citric acid in an immersion plating bath consisting of Rochelle salts, copper, nickel and stannous salts.

## EXAMPLE 6

|                            | Specific Example, Percent | Specific Dry Admixture, Percent |
|----------------------------|---------------------------|---------------------------------|
| Citric acid                | 5.0                       | 47.6                            |
| Succinic anhydride         | 1.0                       | 9.5                             |
| Copper sulfate             | 1.0                       | 9.5                             |
| Nickel sulfate             | 3.0                       | 28.6                            |
| Stannous chloride (anhyd.) | 0.5                       | 4.8                             |
| Water                      | 89.5                      |                                 |
|                            | 100.0                     | 100.0                           |

## EXAMPLE 7

|                            | Specific Example, Percent | Specific Dry Admixture, Percent |
|----------------------------|---------------------------|---------------------------------|
| Rochelle salt              | 5.0                       | 47.6                            |
| Citric acid                | 1.0                       | 9.5                             |
| Copper sulfate             | 1.0                       | 9.5                             |
| Nickel sulfate             | 3.0                       | 28.6                            |
| Stannous chloride (anhyd.) | 0.5                       | 4.8                             |
| Water                      | 89.5                      |                                 |
|                            | 100.0                     | 100.0                           |

## EXAMPLE 8

|                                | Specific Example, Percent | Specific Dry Admixture, Percent |
|--------------------------------|---------------------------|---------------------------------|
| Rochelle salt                  | 5.0                       | 46.3                            |
| Hydroxyacetic acid (70% soln.) | 1.3                       | 12.0                            |
| Copper sulfate                 | 1.0                       | 9.3                             |
| Nickel sulfate                 | 3.0                       | 27.8                            |
| Stannous chloride (anhyd.)     | 0.5                       | 4.6                             |
| Water                          | 89.2                      |                                 |
|                                | 100.0                     | 100.0                           |

Additional examples in which succinic anhydride or diglycolic acid are employed are:

## EXAMPLE 9

|                            | Specific Example, Percent | Specific Dry Admixture, Percent |
|----------------------------|---------------------------|---------------------------------|
| Boric acid                 | 5.0                       | 47.6                            |
| Succinic anhydride         | 1.0                       | 9.5                             |
| Nickel sulfate             | 3.0                       | 28.6                            |
| Copper sulfate             | 1.0                       | 9.5                             |
| Stannous chloride (anhyd.) | 0.5                       | 4.8                             |
| Water                      | 89.5                      |                                 |
|                            | 100.0                     | 100.0                           |

## EXAMPLE 10

|                            | Specific Example, Percent | Specific Dry Admixture, Percent |
|----------------------------|---------------------------|---------------------------------|
| Boric acid                 | 5.0                       | 47.6                            |
| Diglycolic acid            | 1.0                       | 9.5                             |
| Nickel sulfate             | 3.0                       | 28.6                            |
| Copper sulfate             | 1.0                       | 9.5                             |
| Stannous chloride (anhyd.) | 0.5                       | 4.8                             |
| Water                      | 89.5                      |                                 |
|                            | 100.0                     | 100.0                           |

I have found in my experiments that certain combinations of previously known complexing and modifying agents afford improvement over the agents as used singly. This is demonstrated in Example 7 (above) by citric acid and Rochelle salt in a tertiary copper-nickel-tin bath; and in a further example herein by citrate and ethylene diamine tetraacetate (Versene) in a binary copper-tin bath.

Since the electrolytes of my invention are useful, with modifications, to be employed for the plating of less than three plating metals, I have reduced to practice such modification, and detail a boric acid-containing formula, as below:

## EXAMPLE 11

|                            | Specific Example, Percent | Specific Dry Admixture, Percent |
|----------------------------|---------------------------|---------------------------------|
| Sodium citrate             | 1.5                       | 25.0                            |
| Versene                    | 1.0                       | 16.7                            |
| Copper sulfate             | 1.0                       | 16.7                            |
| Stannous chloride (anhyd.) | 1.0                       | 16.7                            |
| Sodium glycolate           | 0.5                       | 8.2                             |
| Sodium chloride            | 1.0                       | 16.7                            |
| Sulfuric acid (by volume)  | 0.5                       |                                 |
| Water                      | 93.5                      |                                 |
|                            | 100.0                     | 100.0                           |

## Example 12

|                    | Specific Example, Percent | Specific Dry Admixture, Percent |
|--------------------|---------------------------|---------------------------------|
| Copper sulfate     | 3.0                       | 87.73                           |
| Thiourea           | 0.06                      | 1.75                            |
| Sulfuric acid      | 3.0                       |                                 |
| Boric acid         | 0.3                       | 8.77                            |
| Glutaric anhydride | 0.06                      | 1.75                            |
| Water              | 93.58                     |                                 |
|                    | 100.00                    | 100.00                          |

Adherence of the plated coating was excellent at 8.4 and 10.0% iron.

A further binary metal plating formula is as follows, employing succinic acid:

## Example 13

|                | Specific Example, Percent | Specific Dry Admixture, Percent |
|----------------|---------------------------|---------------------------------|
| Boric acid     | 5                         | 50                              |
| Succinic acid  | 1                         | 10                              |
| Nickel sulfate | 3                         | 30                              |
| Copper sulfate | 1                         | 10                              |
| Water          | 90                        |                                 |
|                | 100                       | 100                             |

While I have indicated the preferred grades, for best results, other grades may be substituted, such as are well known in the art.

My reduction to practice of the above concepts may be summarized by a generalized formulation of the nature:

Preferred range of concentrations in solution (by weight):

Electroplating salt or salts 0.01 to 10%.  
Complexing and chelating agent 0.5 to 10%.  
Enhancing and modifying agent 0.01 to 5%.

Brightening agents were evaluated in the following bath:

|                            | Percent |
|----------------------------|---------|
| Boric acid                 | 4       |
| Citric acid                | 2       |
| 5 Nickel sulfate           | 3       |
| Copper sulfate             | 1       |
| Stannous chloride (anhyd.) | 0.5     |

The preferred concentration ranges in solution were:

|    |                                |                             |
|----|--------------------------------|-----------------------------|
| 10 | Magnesium chloride             | 0.25 to 1.5%.               |
|    | Benzimidazole                  | 0.05 to 0.5%.               |
| 15 | 2-methylbenzimidazole          | 0.05 to 0.5%.               |
|    | 2-methylpiperazine (70% soln.) | 0.01 to 0.25%.              |
|    | 2-butyne-1, 4-diol             | 0.1 to 0.25% or saturation. |
|    | Paraformaldehyde               | 0.01 to 0.2% or saturation. |
|    | 3-amino-1H-1,2,4-triazole      | 0.01 to 0.25%.              |
| 20 | Sodium acetate                 | 0.01 to 1% or saturation.   |
|    | Sodium formate                 | 0.01 to 1% or saturation.   |
|    | Sodium fluoroborate            | 0.01 to 1% or saturation.   |

As an addition to the above generalized formulation, the optional brightening agent range may be 0.001 to 1%.

By the term "complexing and chelating agent" in the 25 claims, is meant one that exhibits chemical sequestering characteristics added to chelating characteristics which affect the metal salts during plating. "Enhancing and modifying agent" is one that affects the complexing and chelating agent so that the desirable results described in the 30 fourth paragraph of this specification are achieved. By the term "brightening agents" is meant materials whose principal function in the plating bath seems to be to improve the appearance of the deposited coating, by imparting luster or brightness to the coating.

35 The actual steps in employing in immersion electroplating by the use of the new electrolytes of this invention are those generally used in the art.

In the above examples, the nickel sulfate is preferably the material termed hexahydrate ( $6\text{H}_2\text{O}$ ) and the copper 40 sulfate is preferably the material termed pentahydrate ( $5\text{H}_2\text{O}$ ).

What is claimed is:

1. An immersion process for applying a brasslike "liquor finish" to steel which comprises immersing steel 45 in an aqueous solution containing from about 0.01% to about 10% by weight of a water soluble salt of copper, nickel, and tin, from about 0.5% to about 10% of a complexing agent which is a member of a group consisting of boric acid and citric acid, and from about 0.01% to about 50 5% of an enhancing agent which is a member of the group consisting of glutaric acid, succinic acid, and glycolic acid, their anhydrides and water soluble salts.

2. A process as in claim 1 where the complexing agent is boric acid and the enhancing agent is glutaric anhydride.

3. A process as in claim 1 where the complexing agent is boric acid and the enhancing agent is sodium glycolate.

4. A process as in claim 1 where the complexing agent is boric acid and the enhancing agent is succinic acid.

5. A process as in claim 1 where the complexing agent 60 is citric acid and the enhancing agent is sodium glycolate.

6. A composition comprising a mixture of dry ingredients suitable for addition to water to prepare an immersion coating solution for steel objects comprising on a parts by weight basis from about 5% to about 10% of a 65 water soluble copper salt, from about 25% to about 30% of a water soluble nickel salt, from about 3% to about 5% of a water soluble tin salt, from about 25% to about 50% of a complexing agent selected from a group of boric and citric acids, and from about 10% to about 25% of an enhancing agent selected from a group consisting of the free acid, its salt, or the anhydride of glutaric, succinic, and glycolic acids.

7. A composition as in claim 6 where the complexing agent is boric acid and the enhancing agent is glutaric anhydride.

8. A composition as in claim 6 where the complexing agent is boric acid and the enhancing agent is sodium glycolate.

9. A composition as in claim 6 where the complexing agent is boris acid and the enhancing agent is succinic acid.

10. A composition as in claim 6 where the complexing agent is citric acid and the enhancing agent is sodium glycolate.

## References Cited

10

| UNITED STATES PATENTS |         |                         |
|-----------------------|---------|-------------------------|
| 570,554               | 11/1896 | Jordis 204—44           |
| 2,081,630             | 5/1937  | Leonard 106—1 XR        |
| 3,346,404             | 10/1967 | Gardner et al. 106—1 15 |
| 1,837,835             | 12/1931 | Pinner et al. 204—43-XR |
| 2,411,674             | 11/1946 | Wilson 204—52           |
| 2,437,865             | 3/1948  | Stareck 204—52          |
| 2,653,128             | 9/1953  | Brenner et al. 204—43   |
| 2,773,818             | 12/1956 | Moy et al. 204—49 20    |
| 2,882,208             | 4/1959  | Becking et al. 204—49   |

|             |         |                         |
|-------------|---------|-------------------------|
| 3,032,486   | 5/1962  | Sallo et al. 204—43     |
| 3,149,057   | 9/1964  | Parker et al. 204—43 XR |
| 3,149,058   | 9/1964  | Parker et al. 204—43 XR |
| 3,211,578   | 10/1965 | Gutzeit 106—1           |
| 5 3,380,898 | 4/1968  | Danemark et al. 204—44  |

## FOREIGN PATENTS

|              |        |                |
|--------------|--------|----------------|
| 1,162,398    | 9/1958 | France.        |
| 871,276      | 6/1961 | Great Britain. |
| 10 1,006,333 | 9/1965 | Great Britain. |

## OTHER REFERENCES

IBM Technical Disclosure Bulletin, vol. 4, No. 11, p. 10, April 1962.

JOHN H. MACK, Primary Examiner

G. L. KAPLAN, Assistant Examiner

U.S. Cl. X.R.

117—130; 204—44, 45